

# United States Patent Office

3,135,579

Patented June 2, 1964

1

3,135,579

## TREATMENT OF TEXTILE FABRICS WITH DIEPOXYDIOXANES

Arnold M. Sookne, Silver Spring, and John H. Margeson, West Hyattsville, Md., and Howard R. Guest, Charleston, and Joe T. Adams, St. Albans, W. Va., assignors to Union Carbide Corporation, a corporation of New York

No Drawing. Filed May 21, 1962, Ser. No. 196,476  
9 Claims. (Cl. 8—116)

This invention relates to an improved process for the treatment of cellulosic textile materials to impart shrink and crease resistant features. In one aspect, this invention relates to the treatment of cellulosic and cellulosic-containing textile fabrics with diepoxydioxanes. The more recent developments of new finishes for cellulosic and cellulosic-containing fabrics have been directed to the polyepoxides which can be applied to the fabrics in various aqueous or emulsified forms and thereafter cured within the fibers by means of an epoxy curing agent. While these new finishes are an improvement over the nitrogen-containing products, they are still subject to certain deficiencies. The use of a softener is required in many cases to overcome the harsh feel imparted to the fabric by the polyepoxide finish and additionally, the yellowing of the softener itself during the curing stage may necessitate the use of a bleach. While a few of the polyepoxides are slightly soluble in water, their solubility is such that it is not advantageous to prepare treating baths of such low concentrations since it would necessitate repeated padding to obtain the desired add-on of polyepoxide. For these reasons an emulsifying agent or non-aqueous solvent is usually required in order to prepare a bath of suitable concentration. This is particularly evident when polyepoxide polymers of high molecular weight are used. The use of non-aqueous solvents to circumvent the low solubility in water of the polyepoxide finishes also creates plant operating problems which detract from their other advantages.

A further disadvantage noted in the use of the polyepoxides to impart wash-and-wear properties is their inability to be sufficiently resistant to acid hydrolysis to tolerate the presence of the strong acid catalysts which are used conventionally for curing formaldehyde on cellulose. Previous attempts to employ polyepoxides in combination with formaldehyde have largely been disappointing due to the acid hydrolysis of the polyepoxide.

Accordingly, one or more of the following objects will be achieved by the practice of the instant invention. It is an object of the present invention to provide a novel process for the treatment of cellulosic and cellulosic-containing textile materials wherein the disadvantages previously indicated are substantially eliminated. It is also an object of the present invention to provide a process for impregnating cellulosic and cellulosic-containing textile materials with monomeric polyepoxides whereby the material is rendered both shrink and crease resistant, while imparting to the material after laundering, a soft, smooth finish without ironing. A further object of the present invention is to provide a process for treating textile fabrics which will not exhibit undesirable chlorine retention properties and which are durable to laundering. Another object is to provide a process for treating textile materials with a polyepoxide which does not require the use of emulsifying agents or non-aqueous solvents. A further object of the present invention is to provide textile treating solutions containing a novel polyepoxide which when applied to a textile fabric can be cured quickly and at low temperatures. Another object is to provide a process for treating textile materials with a polyepoxide which is resistant to acid hydrolysis and can be employed in combi-

2

nation with formaldehyde. A further object of this invention is to provide a process for treating textile materials with diepoxydioxanes. A still further object is to provide a process for treating textile materials with 2,3-bis(2,3-epoxy-propoxy)-1,4-dioxane. These and other objects will readily become apparent to those skilled in the art in the light of the teachings herein set forth.

In its broad aspect, this invention is directed to a process for treating cellulosic and cellulosic-containing textile materials whereby the material is rendered both shrink and crease resistant while imparting to the material after laundering a soft, smooth finish without ironing which comprises impregnating the textile material with a diepoxydioxane. Thereafter the material is heated to promote the reaction of the polyepoxide with the fabric and thereby impart the shrink and crease resistant features.

Although the concept of imparting wash-and-wear properties to cellulosic fabrics by the treatment with polyepoxides is not new, the improvement embodied in the present invention is both unique and outstanding. Heretofore, numerous nitrogen-containing finishes and polyepoxides have been investigated for their ability to impart wash-and-wear properties to textile fabrics, yet none has been found to date which gives an essentially "as ironed" appearance which is durable for the life of the garment. Previous attempts to impart permanent wash-and-wear properties have, for the most part, been disappointing. As the fabrics treated with nitrogen-containing finishes were repeatedly laundered, they would be accompanied by a marked decrease in crease resistance. With many commercially available nitrogenous finishes, this deficiency was noticeable even after as few as two or three launderings.

A further unique advantage of the polyepoxides used in the process of this invention is their resistance to acid hydrolysis. This feature renders the polyepoxide especially attractive for use in blends with formaldehyde which is cured conventionally by strong acid catalysts. Inasmuch as formaldehyde itself is a highly efficient and inexpensive cross-linking agent a more efficient and economical treatment can be employed to impart the desired wash-and-wear properties to textile fabrics. Moreover, it has been found that fabrics treated with the aforementioned polyepoxides and formaldehyde possess properties superior to those obtained using the same amount of either of the components separately. For instance, a significantly lower loss of fabric strength was found than when formaldehyde was employed as the sole reactant. Additionally, a higher crease recovery and wash-and-wear index was obtained than when the polyepoxide was employed alone. It is thus possible to acquire an excellent combination of functional properties for wash-and-wear use at a substantially lower add-on of polyepoxide and formaldehyde, i.e. about 6 weight percent than for the individual components of the blend.

The diepoxydioxanes which are suitable for use in the practice of the instant invention are the bis(epoxyalkoxy)-dioxanes represented by the following formula:



wherein R represents a divalent hydrocarbon radical of from 1 to 3 carbon atoms, and R<sub>1</sub> represents a monovalent radical selected from the group consisting of hydrogen and methyl. Illustrative compounds which can be employed include,

2,3-bis(2,3-epoxypropoxy)-1,4-dioxane,  
2,5-bis(2,3-epoxypropoxy)-1,4-dioxane,

2,3-bis(2-methyl-2,3-epoxypropoxy)-1,4-dioxane,  
 2,5-bis(2-methyl-2,3-epoxypropoxy)-1,4-dioxane,  
 2,3-bis(3,4-epoxybutoxy)-1,4-dioxane,  
 2,5-bis(3,4-epoxybutoxy)-1,4-dioxane,  
 2,3-bis(3-methyl-3,4-epoxybutoxy)-1,4-dioxane,  
 2,5-bis(3-methyl-3,4-epoxybutoxy)-1,4-dioxane,  
 2,3-bis(4,5-epoxybutoxy)-1,4-dioxane,  
 2,5-bis(4,5-epoxybutoxy)-1,4-dioxane,  
 2,3-bis(4-methyl-4,5-epoxybutoxy)-1,4-dioxane, and  
 2,5-bis(4-methyl-4,5-epoxybutoxy)-1,4-dioxane.

The diepoxydioxanes are prepared by the reaction of the corresponding diolefinic diether dioxane precursor, i.e., the bis(alkenylloxy)dioxane, with an organic peracid. Among the peracids contemplated include, for example, the aliphatic peracids, the cycloaliphatic peracids, the aromatic peracids, and the like. The organic hydrocarbon peracids are preferred. Illustrative peracids include, for instance, peracetic acid, perpropionic acid, perbutyric acid, perhexanoic acid, perdodecanoic acid, perbenzoic acid, monoperphthalic acid, and the like. The lower aliphatic hydrocarbon peracids which contain from 2 to 4 carbon atoms are highly suitable. Peracetic acid is most preferred. It is highly desirable to employ the peracid as a solution in an inert normally liquid organic vehicle such as ethyl acetate, butyl acetate, acetone and the like. A solution comprising from about 10 to about 50 weight percent of peracid, based on the total weight of peracid and inert organic vehicle is suitable; from about 20 to 40 weight percent is preferred. The epoxidation reaction can be conducted at a temperature in the range of from about 0° C., and lower, to about 100° C., and higher, and preferably from about 25° to about 75° C. It is highly desirable to employ an excess of the stoichiometric quantity of peracid (per carbon to carbon double bond of the diolefinic diether precursor) in order to effect or favor substantial diepoxidation of said precursor. For instance, from about 2.2 to about 10, and higher mols of peracid per mol of diolefinic diether precursor can be employed with advantageous results. The epoxidation reaction is conducted for a period of time sufficient to introduce oxirane oxygen at the site of the carbon to carbon double bonds present in the diolefinic diether precursor, e.g., from several minutes to several hours. Periodic analysis of samples of the reaction mixture to determine the quantity of peracid consumed during the diepoxidation reaction can be readily performed by the operator by well-known techniques. At the termination of the epoxidation reaction, the unreacted diolefinic diether precursor, acid by-product, unspent peracid, inert vehicle, if employed, and the like, can be recovered from the reaction product mixture, for example, by distillation under reduced pressure. Further well-known purification techniques can be employed, as desired.

The diolefinic diether precursor can be prepared by the reaction of 2,3-dichlorodioxane or 2,5-dichlorodioxane with the appropriate monoethylenically unsaturated alcohol or mixtures thereof, preferably in a molar ratio of one mole of dichlorodioxane to at least two mols of monoethylenically unsaturated alcohol. This reaction readily proceeds at room temperature, e.g., about 24° C., and the gaseous hydrogen chloride by-product can be continuously removed during the reaction. The desired diolefinic diether precursor can be recovered from the resulting reaction product mixture via conventional techniques such as distillation, fractionation, crystallization, and the like.

The 2,3-dichlorodioxane reagent can be prepared by reaction of dioxane and chlorine gas, at elevated temperatures, e.g., about 70° to 100° C., in the absence or presence of a catalyst, e.g., stannous chloride. Thereafter, nitrogen gas can be bubbled through the resulting reaction product mixture to remove any unreacted chlorine, if desired. Unreacted dioxane can be removed from said reaction product mixture by conventional means, e.g., distillation under reduced pressure, thus giving 2,3-dichlorodioxane.

The 2,5-dichlorodioxane reagent can be prepared by the

reaction of dioxane and chlorine gas, at relatively low temperatures, e.g., about -30° C. to about 0° C., generally in the presence of an inert normally liquid organic vehicle, e.g., carbon tetrachloride. The resulting reaction product mixture then can be cooled in a Dry Ice bath which causes 2,5-dichlorodioxane to crystallize from said reaction product mixture. The 2,5-dichlorodioxane is readily recovered therefrom via well-known techniques, e.g., crystallization.

In practice, the objectives of the present invention can best be achieved by impregnating the fabric with an aqueous medium containing the bis(epoxyalkoxy)dioxane and a curing catalyst. Impregnation is effected by a conventional padding operation. Thereafter the fabric is dried at a low temperature and then cured at a temperature sufficient to promote the reaction of the polyepoxide with the cellulose.

By applying the polyepoxide of this invention to textile fabrics the disadvantages inherent in the past have been overcome to give a fabric which is soft, white, and has a high degree of crease recovery, and shrink resistance. The cellulosic textile fabrics treated by the process of this invention retain these properties well after repeated laundering and are not subject to chlorine retention. Both whiteness and the original strength of the fabrics are retained to a surprisingly high degree. Treatment by this method represents a substantial improvement over other finishes heretofore available.

Application of the polyepoxide to the fabric is best effected from an aqueous medium. The term "aqueous medium" as used throughout the specification and claims is intended to encompass textile treating solutions wherein the solvent medium is solely water, mixtures of water and emulsifying agents, or mixtures of water and organic solvents miscible with water. While the polyepoxide finishes generally in use are not easily dispersed in an aqueous treating bath to give a homogeneous solution because of a low degree of water solubility, the bis(epoxyalkoxy)-dioxanes, particularly 2,3-bis(2,3-epoxypropoxy)-1,4-dioxane have a distinct advantage of being miscible in most all proportions with water at 25° C. so that solvents or emulsifying agents are not necessary in preparing the treating bath. This is of particular value in view of the trend in textile finishing operations to use the minimum wet pick-up that is possible with modern pad rolls. Operating in this manner permits more rapid production in the drying and curing stages since only small amounts of water need to be evaporated. 2,3-bis(2,3-epoxypropoxy)-1,4-dioxane is ideally suited for this improved technique since it is completely soluble in water in all proportions. It is therefore possible to prepare a 30 weight percent solution of this diepoxide and pad onto the fabric at a 70 percent wet pick-up and obtain a 21 weight percent add-on. The majority of polyepoxides do not possess sufficient water solubility to permit the preparation of solutions of such a high concentration.

The use of emulsifying agents or organic solvents may be needed, however, in those instances when water insoluble components are added to the textile treating solution. Among the emulsifying agents and solvents which can be employed if required are methylcellulose, hydroxyethylcellulose, carboxymethylcellulose, sodium alginate, polyvinyl alcohol, polyethylene oxide, toluene, xylene, the lower aliphatic alcohols such as ethyl alcohol, butyl alcohol, isopropyl alcohol, acetone, esters, and the like. The concentration of emulsifying agent is not necessarily critical and can vary in amounts from about 0.1 to 15 percent of the solution.

While the curing step can be accomplished by heating, it can be accelerated by the use of a suitable curing catalyst. The catalysts employed are the so-called "acid-acting" curing agents or epoxy curing agents which include not only acids but compounds capable of acting as acids, such as acidic salts, Lewis acids, and the like. Examples of the acid-acting or epoxy curing agents in-

clude, among others, organic and inorganic acids and their anhydrides, such as phosphoric acid, hydrochloric acid, boric acid, the alkane sulfonic acids, perchloric acid, persulfuric acid, p-toluenesulfonic acid, citric-acid, acetic acid, acetic acid anhydride, butyric acid, caproic acid, phthalic acid, phthalic acid anhydride, tartaric acid, oxalic acid, succinic acid, succinic acid anhydride, fumaric acid, glutamic acid, malonic acid, acetoacetic acid, and naphthalic acid; metal salts such as the fluoroborates of magnesium, tin, cadmium and sodium as well as zinc, boron trifluoride etherate, stannic chloride, aluminum chloride, magnesium chloride, sodium sulfate, zinc sulfate, and aluminum sulfate, and amine hydrohalides such as hydrochlorides of aniline, benzylidene, n-propylamine, di-n-butylamine, di-benzylamine, triethylamine, alpha-phenylethylamine, alpha-naphthylamine, beta-aminoanthraquinone, 1,3-diaminoanthraquinone, piperidine, pyridine, quinoline, morpholine, pyrrole and guanidine, and hydrochlorides of hydroxyamines as 2-amino-2-methylpropanol and isobutanol amine. The amount of catalyst employed is not necessarily critical and can vary in amount from about 0.01 percent to about 10 percent by weight, with a preferred range of from about 0.1 percent to about 5 percent.

The optimum amount of polyepoxide to be applied to the textile material is an amount sufficient to give a desired wash-and-wear rating of 4 or 5 as hereinafter indicated. A preferred method is to immerse the fabric in an aqueous medium containing from about 1 to about 30 percent by weight of the polyepoxide, and from 0.01 to 10 percent of the curing catalyst and then pass it through a squeeze roller. A second immersion and squeezing can be effected if necessary, leaving the fabric impregnated with approximately 60 to 100 percent of its own weight of solution. After this padding procedure, the fabric is mounted on a pin frame and dried at relatively low temperatures to remove water. While drying may be accomplished by allowing the fabric to remain in contact with the air, a temperature range of from about 95° F. to about 175° F. for 5 to 1 minutes is preferred. Since the drying time is not critical, a wider range of drying temperature can be employed equally as well.

Upon drying, the fabric is "cured" at a temperature sufficient to promote the reaction of the polyepoxide with the fibrous material being treated. Temperatures from about 240° to about 400° F. and more preferably from about 275° F. to about 350° F. can be employed for periods ranging from about 15 seconds to about 5 minutes, with the higher temperatures using the shorter curing period. After the curing step, the fabric is scoured to remove unreacted polyepoxide or epoxy curing catalyst. Scouring is effected by washing in hot water (approximately 170° F.) containing a small quantity of detergent. The scouring conditions themselves are not critical as long as unreacted material is removed from the fabric. After scouring, the fabric is dried and evaluated.

In another aspect of the present invention, the textile treating solutions can include mixtures of one or more polyepoxides and one or more known textile finishes, including the nitrogen-containing finishes, either alone or in the presence of an epoxy curing catalyst. The undesirable yellowing effect of the nitrogenous textile resins after chlorine bleaching when such resins are used as the sole finish for white goods, is eliminated or greatly reduced when employed in conjunction with polyepoxides. Excellent results are obtained, for example, by the use of the instant polyepoxide in conjunction with the melamine-formaldehyde resins, 1,3-dimethylol-5-ethyltetrahydro-5-triazin-2(1H)-one; mono- and dimethylol ureas, mono- and dimethylol ethylene ureas, methylated methylol ureas, and the like.

As previously indicated, the use of blends of the bis(epoxyalkoxy)dioxane and formaldehyde are of particu-

lar interest for imparting the desired shape-holding properties to textile fabrics. Since the bis(epoxyalkoxy)dioxanes are resistant to acid hydrolysis, they are ideally suited for use in conjunction with the less expensive formaldehyde. Moreover, their combined use has a synergistic effect and imparts a higher degree of crease recovery and breaking strength retention than the use of a comparable amount of each finish alone. In practice when mixtures of the polyepoxide and formaldehyde are employed, the polyepoxide should comprise at least 15 weight percent, and more preferably from about 15 to about 90 weight percent based on the weight of the mixture.

The textile treating solution employed for imparting the wash-and-wear characteristics to the cellulosic or cellulosic-containing materials can also contain, in addition to the aforementioned polyepoxides, plasticizers, natural resins, textile softening agents and the like.

The cellulosic textile fabrics used to illustrate the process of this invention were 80 x 80 cotton print cloth and 80 x 80 staple rayon fabric. The fabric was white, had been scoured and bleached, and was in suitable condition for application of resin treatment.

In the evaluation of the properties of the treated fabric, the following tests were conducted.

(a) Breaking strength; measured by the raveled strip method. American Society for Testing Materials D39-49 (warp direction only).

(b) Crease recovery; measured with the Monsanto tester. American Society for Testing Materials D1295-53T (warp direction only). By this test the ability of a fabric to recover from a crushing fold is measured.

(c) Dimensional stability; American Association of Textile Chemists and Colorists, tentative test method 40-52.

(d) Wash-and-wear evaluation; by means of the following scale, the wash-and-wear properties of the treated material were evaluated.

| Scale: | Evaluation      |
|--------|-----------------|
| 5      | As ironed.      |
| 4      | Wearable.       |
| 3      | Needs ironing.  |
| 2      | Not acceptable. |
| 1      | Very wrinkled.  |

Ref.: Textile Research Journal, 26, 974 (1956); American Dyestuff Reporter, 48, 37 (1959).

(e) Color; the yellowness of the treated fabric was determined by comparison with the original bleached fabric. The yellowness index was determined using a Hunter multipurpose reflectometer. This abridged spectrophotometer employs three filters in measuring the 45°, 0° reflectance of a fabric with respect to amber, green and blue light. A simple yellowness index is provided by

$$55 \quad \text{Yellowness} = \frac{A - B}{G}$$

where A, B and G represent the reflectances in amber, blue and green light, respectively. The index so obtained correlates closely with subjective evaluations. A white fabric has a yellowness which approaches zero, while an index in the range of 0.2 or 0.3 describes a very yellow sample.

(f) Dry add-on; determined by measuring the increase in weight of the fabric after treatment with the polyepoxide, and scouring to remove unreacted material; is a measurement of the total epoxide which had reacted with the fiber.

The term "cellulosic and cellulosic-containing textile materials" as used throughout the specification and claims is intended to include cellulose or cellulose-containing fibers, whether in the finished state or at some intermediate stage in processing; cellulose and cellulose-containing fabrics whether woven or knitted; and garments or other articles made from such fabrics. Thus, materials containing cellulose, regenerated cellulose, and mixtures of

the two are intended to be within the scope of the present invention.

The following examples are illustrative. Unless otherwise indicated, all percentages of ingredients are by weight:

#### EXAMPLE 1

##### *Preparation of 2,3-Bis(2,3-Epoxypropoxy)-1,4-Dioxane*

A. *Preparation of 2,3-diallyloxy-1,4-dioxane*.—A mixture of 872 grams of an aqueous glyoxal solution (containing 26.6 weight percent glyoxal and 8.8 weight percent ethylene glycol), 170 grams of ethylene glycol, 696 grams of allyl alcohol, and 3 grams of sulfuric acid was charged to the kettle of a still which was fitted with a decanting head. The mixture was boiled under reflux until the theoretical amount of water was removed overhead using 600 milliliters of benzene as the azeotroping agent. The catalyst was then neutralized with sodium acetate and the mixture rapidly distilled to give, after removal of the low-boiling materials, 400 grams of product having a boiling point of 83°–92° C. at a pressure of 3 millimeters of mercury. Redistillation of the product gave 310 grams of 2,3-diallyloxy-1,4-dioxane having a boiling point of 75°–77° C. at a pressure of 0.6 millimeters of mercury, and a refractive index,  $N_D^{30}$  of 1.4549.

B. *Epoxidation of 2,3-diallyloxy-1,4-dioxane*.—To 225 grams of 2,3-diallyloxy-1,4-dioxane which was maintained in a kettle with stirring at 60° C. there was added dropwise over a period of two hours and forty-five minutes 998 grams of a 24.3 percent solution of peracetic acid in ethyl acetate. After an additional four hours at 60° C. the reaction was 93 percent complete as indicated by a titration of the solution for peracetic acid. After standing overnight at 0° C., the volatiles were removed by co-distillation with 1450 grams of ethylbenzene and the residue distilled through an 8 inch x 32 millimeter glass helices-packed column to give 8 grams of heads cut, 24 grams of 2-allyloxy-3-(2,3-epoxypropoxy)-1,4-dioxane and 221 grams of 2,3-bis(2,3-epoxypropoxy)-1,4-dioxane having a boiling point of 125°–140° C. at a pressure of 0.25 millimeters of mercury, and a refractive index,  $N_D^{30}$  of 1.4632–1.4683. Redistillation of the diepoxide gave a product with the following properties: boiling point 140° C. at a pressure of 0.25 millimeters of mercury; refractive index,  $N_D^{30}$  1.4678; and a purity of 97 percent by epoxide analysis (pyridine hydrochloride method).

Upon analysis the diepoxide had the following composition. Calculated for  $C_{10}H_{16}O_6$ : C, 51.72; H, 6.94. Found: C, 51.79; H, 6.87.

In an analogous manner the 2,5-bis(2,3-epoxypropoxy)-1,4-dioxane is prepared from 2,5-diallyloxy-1,4-dioxane.

#### EXAMPLE 2

A treating solution was prepared containing 12.5 weight percent of bis-2,3-(2,3-epoxypropoxy)-1,4-dioxane, 1.25 percent zinc fluoborate and the remainder water. A sample of 80 x 80 cotton print cloth was immersed in this solution, padded to a wet pick-up of approximately 85 percent of the fabric weight, air dried for three minutes at 167° F. and then cured for three minutes at 248° F. The treated fabric was then laundered with a 0.1 percent solution of a built detergent to remove residual reagents, tumble dried, and evaluated according to the methods described above. The dry add-on after laundering was found to be 9.2 percent. The fabric had a wash-and-wear index of 5—, a dry and wet crease recovery of 76 and 73 percent respectively, a yellow index of 0.04 and a breaking strength retention of 54 percent.

The original untreated fabric was immersed in water, dried and found to have a wash-and-wear index of 1, dry and wet crease recoveries of 43 and 41 percent respectively and yellowness index of 0.03.

#### EXAMPLE 3

A treating solution was prepared containing 15.0 weight percent of bis-2,3-(2,3-epoxypropoxy)-1,4-dioxane, 1.25

percent zinc fluoborate, and the remainder water. A sample of 80 x 80 cotton print cloth was immersed in this solution, padded to a wet pick-up of approximately 82 percent of the fabric weight, air dried for three minutes at 167° F. and then cured for three minutes at 248° F. The treated fabric was then laundered with a 0.1 percent solution of a built detergent to remove residual reagents, tumble dried, and evaluated according to the methods described above. The dry add-on after laundering was found to be 10.8 percent. The fabric had a wash-and-wear index of 4+, a dry and wet crease recovery of 78 and 73 percent respectively, a yellowness index of 0.04 and a breaking strength retention of 51 percent.

#### EXAMPLE 4

A treating solution was prepared containing 17.5 weight percent of bis-2,3-(2,3-epoxypropoxy)-1,4-dioxane, 1.9 percent zinc fluoborate, and the remainder water. A sample of 80 x 80 cotton print cloth was immersed in this solution, padded to a wet pick-up of approximately 78 percent of the fabric weight, air dried for three minutes at 167° F. and then cured for three minutes at 248° F. The treated fabric was then laundered with a 0.1 percent solution of a built detergent to remove residual reagents, tumble dried, and evaluated according to the methods described above. The dry add-on after laundering was found to be 11.5 percent. The fabric had a wash-and-wear index of 5—, a dry and wet crease recovery of 80 and 76 percent respectively, a yellowness index of 0.04, and a breaking strength retention of 54 percent.

#### EXAMPLE 5

A treating solution was prepared containing 6.0 weight percent of bis-2,3-(2,3-epoxypropoxy)-1,4-dioxane, 1.0 percent zinc fluoborate, and the remainder water. A sample of 80 x 80 cotton print cloth was immersed in this solution, padded to a wet pick-up of approximately 94 percent of the fabric weight, air dried for three minutes at 167° F. and then cured for three minutes at 248° F. The treated fabric was then laundered with a 0.1 percent solution of a built detergent to remove residual reagents, tumble dried, and evaluated according to the methods described above. The dry add-on after laundering was found to be 4.4 percent. The fabric had a wash-and-wear index of 3, dry crease recovery of 64 percent, a yellowness index of 0.02, and a breaking strength retention of 58 percent.

#### EXAMPLE 6

A treating solution was prepared containing 6.0 weight percent of bis-2,3-(2,3-epoxypropoxy)-1,4-dioxane, 0.5 percent zinc fluoborate, and the remainder water. A sample of 80 x 80 cotton print cloth was immersed in this solution, padded to a wet pick-up of approximately 98 percent of the fabric weight, air dried for three minutes at 167° F. and then cured for three minutes at 248° F. The treated fabric was then laundered with a 0.1 percent solution of a built detergent to remove residual reagents, tumble dried, and evaluated according to the methods described above. The dry add-on after laundering was found to be 3.5 percent. The fabric had a wash-and-wear index of 3, a dry crease recovery of 62 percent, a yellowness index of 0.02, and a breaking strength retention of 66 percent.

#### EXAMPLE 7

A treating solution was prepared which contained 1.5 weight percent formaldehyde, 0.5 percent zinc fluoborate and the remainder water. A sample of 80 x 80 cotton print cloth was immersed in this solution, padded to a wet pick-up of approximately 95 percent of the fabric weight, dried for three minutes at 167° F. and cured for three minutes at 248° F. The treated fabric was then laundered with a 0.1 percent solution of a built detergent to remove residual reagents and evaluated as in the preceding examples. The dry add-on after laundering was found to be -0.1 percent. The fabric had a wash-and-

wear index of 3, a crease recovery of 56 percent, a yellowness index of 0.04 and a breaking strength retention of 61 percent.

#### EXAMPLE 8

A treating solution was prepared which contained 6.0 weight percent of bis-2,3-(2,3-epoxypropoxy)-1,4-dioxane, 0.5 percent zinc fluoborate, 1.5 percent formaldehyde and the remainder water. A sample of 80 x 80 cotton print cloth was immersed in this solution, padded to a wet pick-up of approximately 97 percent of the fabric weight, air dried for three minutes at 167° F. and cured for three minutes at 248° F. The treated fabric was then laundered with a 0.1 percent solution of a built detergent to remove residual reagents and evaluated according to the methods used in the preceding examples. The dry add-on after laundering was found to be 3.6 percent. The fabric had a wash-and-wear index of 4, a crease recovery of 71 percent, a yellowness index of 0.03 and a breaking strength retention of 71 percent.

Comparison of the results of Examples 6, 7 and 8 shows that the mixture of 1.5 percent of formaldehyde and 6.0 percent of bis-2,3-(2,3-epoxypropoxy)-1,4-dioxane produced results superior to those obtained when either reagent was used alone. Moreover, it should be noted that the presence of bis-2,3-(2,3-epoxypropoxy)-1,4-dioxane in the treating bath substantially reduced the severe strength loss which resulted from the treatment of cotton with formaldehyde.

#### EXAMPLE 9

A sample 80 x 80 cotton print cloth was treated as described in Example 8. The treated fabric was then subjected to an acid stripping procedure involving immersion in a solution containing 1.5 weight percent of phosphoric acid and 5 percent of urea for five minutes at 170° F. This acid solution which had a pH of 1.9 is capable of stripping most nitrogenous resin treatments from cotton. This treatment also simulates the hydrolytic effects of the acid sour in approximately ten commercial laundries. Prior to the acid stripping procedure the treated cotton had a wash-and-wear index of 4, and a dry crease recovery of 68 percent. After acid stripping the wash-and-wear index was unchanged and the crease recovery was 67 percent. It is therefore evident that the treatment set forth in Example 8 is resistant to acid hydrolysis more severe than that encountered in commercial laundering operations.

#### EXAMPLE 10

A solution containing 15 weight percent bis-2,3-(2,3-epoxypropoxy)-1,4-dioxane, 1 percent zinc fluoborate and the remainder water was allowed to stand at 25° C. and analyzed periodically for epoxide groups. The initial pH of this solution was approximately 3.5. At the end of one hour, more than 99 percent of the original epoxide groups remained, and at the end of four hours 97 percent of the epoxide remained. Thus, under the acidic conditions used in the blend of bis-2,3-(2,3-epoxypropoxy)-1,4-dioxane with formaldehyde hydrolysis of the epoxide in the treating bath does not present any problem.

Although the invention has been illustrated by the preceding examples, the invention is not to be construed as limited to the materials employed therein, but rather, the invention encompasses the generic area as hereinbefore disclosed. Various modifications and embodiments of this invention can be made without departing from the spirit and scope thereof.

What is claimed is:

1. A process for treating cellulosic and cellulosic-containing textile materials whereby said material is rendered both shrink and crease resistant while imparting to said material after laundering a soft smooth finish without ironing which comprises impregnating said textile material with an aqueous medium containing (1) a compound selected from the group consisting of 2,3-bis(vicinal-epoxyalkoxy)-1,4-dioxane and 2,5-bis(vicinal-epoxyalkoxy)-1,4-dioxane, wherein said vicinal-epoxyalkoxy contains from 3 to 5 carbon atoms and wherein the epoxy group is in a terminal position and separated from etheric oxygen by at least 1 carbon atom; and (2) an epoxy curing catalyst; and thereafter drying and heating said impregnated textile material.
2. A process as claimed in claim 1 wherein the textile material is cotton.
3. A process as claimed in claim 1 wherein the textile material is rayon.
4. A process as claimed in claim 1 wherein the textile material is linen.
5. A process for treating cellulosic and cellulosic-containing textile materials whereby said material is rendered both shrink and crease resistant while imparting to said material after laundering a soft smooth finish without ironing which comprises impregnating said textile material with an aqueous medium containing (1) 2,3-bis(vicinal-epoxyalkoxy)-1,4-dioxane wherein said vicinal-epoxyalkoxy contains from 3 to 5 carbon atoms and wherein the epoxy group is in a terminal position and separated from etheric oxygen by at least 1 carbon atom; and (2) an epoxy curing catalyst; and thereafter drying and heating said impregnated textile material.
6. A process for treating cellulosic and cellulosic-containing material whereby said material is rendered both shrink and crease resistant while imparting to said material after laundering a soft, smooth finish without ironing, which comprises impregnating said textile material with an aqueous medium containing from about 1 to about 30 percent by weight, based on said medium, of 2,3-bis(2,3-epoxypropoxy)-1,4-dioxane and from about 0.01 to about 10 percent by weight of an epoxy curing catalyst; and drying and heating said impregnated textile material.
7. A process as claimed in claim 6 wherein the curing catalyst is zinc fluoborate.
8. A process for treating cellulosic and cellulosic-containing textile materials whereby said material is rendered both shrink and crease resistant while imparting to said material after laundering a soft, smooth finish without ironing, which comprises impregnating said textile material with an aqueous medium containing from about 1 to about 30 percent by weight, based on said medium, of a mixture of 2,3-bis(2,3-epoxypropoxy)-1,4-dioxane and formaldehyde, and from about 0.1 to about 10 percent by weight of zinc fluoborate; and drying and heating said impregnated material.
9. A process as claimed in claim 8 wherein the fabric is heated within the temperature range of from about 240° F. to about 400° F. for a period of from about 15 seconds to about 5 minutes, the higher temperatures employing the shorter heating time.

References Cited in the file of this patent

#### UNITED STATES PATENTS

- |    |           |                |                |
|----|-----------|----------------|----------------|
| 65 | 2,993,915 | Luskin         | July 25, 1961  |
|    | 3,054,803 | Robeson et al. | Sept. 18, 1962 |
|    | 3,067,175 | Sullivan       | Dec. 4, 1962   |